

## UNITED STATES PATENT OFFICE.

EDMONDSON WARRIN, OF UPPER MONTCLAIR, NEW JERSEY.

## ENCRUSTED METAL DESIGN ON CERAMIC SUBSTANCES AND PROCESS OF MAKING SAME.

No Drawing.

Application filed June 30, 1920. Serial No. 393,009.

To all whom it may concern:

Be it known that I, EDMONDSON WARRIN, a citizen of the United States, and a resident of Upper Montclair, in the county of Essex and State of New Jersey, have invented a new and Improved Encrusted Metal Design on Ceramic Substances and Process of Making Same, of which the following is a full, clear, and exact description.

10 This invention relates to an encrusted metal design on ceramic substances and process of making same, and has reference more particularly to a ceramic article in which the design is first etched on the article and 15 later coated with various metallic coatings.

This invention also relates to my co-pending application filed January 9, 1920, Serial No. 350,393.

An object of this invention is to provide 20 a process of decorating ceramic substances in which a design, monogram, crest, flag or other decorative motif is first etched on china, glass or other ceramic substances and this etched design is coated with metal in 25 such a way that a full set of dishes can be made, the designs on each of the dishes being exact duplicates regardless of the intricacy of the design. Another object of this 30 invention is to provide a process of decorating china, glass and other ceramic substances which is especially adapted for having a finishing coating of gold on the design.

A still further object of this invention is to provide a process in the class indicated in 35 which a final coating of precious metals such as gold is underlaid with a coating of the base metals such as copper.

In carrying out my process the steps may be broadly classified as (1) covering the article to be etched with an acid resisting composition except where it is desired to have the design etched by the acid. (2) Etching the article in hydrofluoric acid. (3) Coating the design with a metallic paint composition. (4) Firing the metallic paint into the design. (5) Electroplating copper on said design, and (6) electroplating the design with gold.

The first few steps of my process are car-

ried out substantially as described in my 50 aforementioned co-pending application in that the china or glass article is first covered except where the design, monogram, crest, flag or other decorative motif is to be placed, with a waxed preparation composed of 55

|             |          |
|-------------|----------|
| Stearin wax | 25 lbs.  |
| Cresine wax | 100 lbs. |

The desired design, monogram, etc., is engraved, etched, or photoengraved on a plate 60 of steel, copper, glass or lithographic stone and a print is then made therefrom on fine tissue paper using a composition commonly known in the art as a "resist". This resist is a commercial product and is composed 65 principally of

|              |  |
|--------------|--|
| Asphaltum    |  |
| Bees wax and |  |
| Stearin.     |  |

70 The design is printed on the tissue paper by the use of a hand roller, hand, power, or lithographic press, and the printed paper is then applied to the unwaxed part of the article which is being manufactured. After 75 the printed tissue paper is placed in proper position, it is moistened with a solution of six drops of creosote to one pint of water and is gently removed, leaving the acid resisting print adhering to the article being 80 manufactured. Imperfections and connections are then retouched by hand with a decorator's brush using some of same resist to which a small quantity of turpentine is added to make it workable. The article is then 85 placed in a solution of 60% hydrofluoric acid contained in a lead lined tank of suitable size for a period of from ten to twenty minutes according to the depth of etching desired and wherever the article has not been 90 covered with the wax composition or the resist print, the acid will eat into the unprotected surface of the china or glass to approximately one thirty-second of an inch. After the article is removed from the acid 95 the wax composition and the resist print are removed by washing the article in hot water to which a little soda has been added. When

thoroughly dried it is ready for a coat of silver paint applied by hand with a decorator's brush.

The silver paint is commonly used in the art and is composed of the following ingredients:

|    |                                |
|----|--------------------------------|
|    | Metallic silver (precipitated) |
|    | Lead carbonate                 |
| 10 | Potassium carbonate            |
|    | Potassium nitrate              |
|    | Borax (calcined)               |
|    | Powdered flint                 |
|    | Powdered glass.                |

- 15 The metallic silver must be pure and is made so by placing pure silver chloride in a solution containing two parts by weight of concentrated sulphuric acid in seven parts of water. Strips of metallic zinc are then placed in the silver solution and allowed to stand until all the silver is precipitated out of the solution as a grey or brownish solid. This silver is filtered, washed free of the acid as indicated by litmus paper, dried over a sand bath and is then ready for use. The silver chloride is obtained by dissolving metallic silver in a solution of one part of nitric acid in one part of water, precipitating the silver chloride with sodium chloride while the solution is heated on a hot water bath, filtering and washing the silver chloride. The paint ingredients are thinned with turpentine, placed in a paint mill and ground until exceedingly fine, after which most of the surplus turpentine is removed. When using the silver paint the aforementioned ground ingredients are mixed with fat oil or turpentine on a palette with a palette knife until a creamy consistency is obtained and the paint is then applied with a decorator's brush to the article to be decorated. After the article has been painted it is dried in an ordinary heater and when dry is placed in a kiln or muffle and the heat is gradually increased until it reaches 900-1200° F. for glass and 1200-1500° F. for china. When the desired temperature is reached and the silver paint brought to a point where it fuses with the article on which it has been placed, the heater in the kiln or muffle is shut off and the article allowed to gradually cool until the temperature inside the muffle has decreased to about 300° F. and the door is then opened and additional time is allowed for the article to become cool enough to handle.

The fired metallic paint is now scratch buffed and washed clean in water. The article is then suspended from the negative wire in an electric cleaner consisting of

|    |                     |        |
|----|---------------------|--------|
| 60 | Water               | 1 lb.  |
|    | Potassium carbonate | 3 lbs. |
|    | Potassium cyanide   | 8 oz.  |

A current of five to six volts and 180 amperes is used for a period of two or three

minutes. The article is then washed thoroughly and is suspended from the electrode in a copper-plating cell which contains

|                 |           |
|-----------------|-----------|
| Water           | 1 gallon. |
| Sulphuric acid  | 2 oz.     |
| Copper sulphate | 1½ lbs.   |

70

A current of one or two volts and thirty amperes is used for a period of six or seven hours which causes a heavy coating of copper to be deposited on top of the fired silver paint. By suitable modification of the conditions, any of the base metals may be used instead of copper. The article is then sand buffed to take off any rough surfaces and is washed with water containing a small quantity of ammonia.

The copper is now polished until bright and the article is dipped in the aforementioned electric cleaner for the same period of time and with the same conditions. In coating the copper with the layer of precious metals such as gold, the article is wired and suspended from the negative electrode in an electrolytic cell containing the following composition:

|                  |           |
|------------------|-----------|
| Water            | 1 gallon. |
| Chloride of gold | 4 dwts.   |
| Sodium carbonate | 2 oz.     |

95

The solution is heated to 80° C. and a gold anode of 22 or 18 karat is suspended from the negative electrode. A current of three to eight amperes is used and the article is electroplated until the desired amount of gold is deposited on the design. The article is washed and immersed in the aforementioned electric cleaner and again washed. The gold is now polished slightly with rouge.

The purpose of electroplating the copper under the precious metal is for the purpose of economy in the use of the gold and if so desired, the step of electroplating with copper can be eliminated so that the final design is in pure gold at a corresponding increase in cost. By using suitable materials in the final electroplating bath, any desired precious metals such as platinum, silver, etc. may be electroplated over the copper with very good results.

I would state in conclusion that while the example described constitutes a practical embodiment of my invention, I do not limit myself strictly to the details herein described, since, manifestly, the same can be considerably varied without departing from the spirit of the invention as defined in the appended claims.

Having thus described my invention, I claim as new and desire to secure by Letters Patent:

1. A process of decorating china, glass and other ceramic articles with metallic substances which includes the printing with acid resisting printing fluid, the design de-

130

sired to be decorated upon the article, covering the portion of the article not desired to be decorated with an acid resisting compound paste, placing the article in a hydro-  
5 fluoric acid solution, letting the acid eat into the uncovered surface of the article a predetermined depth, filling the eaten portion with a silver solution, fusing the solution to the article, cleaning the fused silver for elec-  
10 troplating, electroplating copper thereon, and electroplating gold on the copper.

2. The process of plating metal to china, glass and other ceramic articles which includes printing the design on the article with

an acid resisting printing fluid, covering the 15 portion of the article not included in the print with an acid resisting compound, drying the fluid and the compound, placing the article in a solution of ceramic eating acid, filling the acid eaten portion with a com- 20 pound of precipitated metallic silver, placing the article in a kiln until the silver com- pound fuses thereon, subjecting the article to an electric cleaning solution, electroplating a copper deposit on the fused compound, and 25 electroplating a gold deposit on said copper deposit.

EDMONDSON WARRIN.